

Feb. 19, 1929.

1,702,837

I. B. MERRIMAN

MANUFACTURE OF RAYON

Filed Nov. 23, 1927

2 Sheets-Sheet 1

*Fig. 1*



*Fig. 2*



*Inventor*  
Isaac B. Merriman  
by Van Everen, Frish  
Hildreth & Cary Atty.

Feb. 19, 1929.

1,702,837

I. B. MERRIMAN

MANUFACTURE OF RAYON

Filed Nov. 23, 1927

2 Sheets-Sheet 2

*Fig. 6*

27



*Fig. 5*



*Fig. 4*



*Investor*  
Isaac B. Merriman  
by Van Ewens Fish  
Heldreth & Cary Atty.

## UNITED STATES PATENT OFFICE.

ISAAC B. MERRIMAN, OF PROVIDENCE, RHODE ISLAND, ASSIGNOR TO MANVILLE JENCKES COMPANY, OF PAWTUCKET, RHODE ISLAND, A CORPORATION OF RHODE ISLAND.

## MANUFACTURE OF RAYON.

Application filed November 23, 1927. Serial No. 235,344.

The present invention relates to rayon (artificial silk) and processes of making rayon and is intended primarily as an improvement in the production of rayon from viscose by the pot spinning process, although in certain aspects the invention is applicable to the production of rayon from other substances and by other spinning processes.

In the pot spinning method of manufacturing rayon at present in use, a cellulose solution such as viscose, is precipitated in the form of slender fibrous filaments by forcing the solution through a spinneret into a precipitating or setting bath. The filaments are then gathered together to form a thread and the thread is guided to a centrifuge pot by which it is twisted and formed into a so-called "cake". From the "cake", after being removed from the pot, the thread is wound on reels to form skeins which are then subjected to a series of operations to prepare the rayon for commercial use. These subsequent operations on the thread while in skein form contribute a large part of the expense in the manufacture of rayon not only because of the time and labor required, but also because of the difficulty of handling the thread in this form and the waste of material resulting from the necessarily harsh treatment to which the skeins are subjected. The skeins, as taken from the reels, are ordinarily separated into a number of smaller skeins to prevent tangling, and the skeins so formed are usually then washed, dried, and thereafter subjected to a desulphurizing operation for removing chemicals brought over from the original cellulose solution. The skeins of thread may be bleached and oiled and after again being dried are ready for use as white or uncolored rayon. Where colored material is desired, it is usually dyed after the last drying operation, either in the skein or subsequent to the weaving of the rayon into cloth.

The process as described above is open to many disadvantages, not only because of the expense of manufacture, but also because of the quantity of waste and inferior thread produced. The skeins, which consist of bundles of loose threads, must be carefully handled to prevent tangling and the various solutions used for washing, bleaching, etc., must be applied with great care, either by dipping or by light spraying, in order to pre-

vent breaking down of the delicate fibers, secure uniform penetration of the various treating liquids, and an even absorption of the dyes. Moreover, in order to impart luster to the thread, it is necessary to stretch it during some step in the process and this operation is ordinarily carried out by putting the skeins under tension during the first drying step. This results in broken filaments and consequently in the production of thread of inferior grades.

The principal object of the present invention is to devise a method for the manufacture of rayon which is, as compared with present day methods, simple and inexpensive, which results in the production of thread of high strength and luster and uniform color, and which avoids the breakage of filaments at any stage in the treatment and the production of thread which must be graded as inferior from this cause.

Another object of the invention is to provide a package of precipitated fiber in a condition to permit convenient and rapid operations of bleaching, dyeing, and the like with substantially uniform effect upon all parts of the fiber and with little danger of breakage or other mechanical injury.

A still further object of the present invention is to produce rayon of high strength and possessing the desirable characteristics of luster and color which are uniform throughout the product.

With these and other objects in view as will hereinafter appear, the principal feature of the present invention comprises a method by which all operations subsequent to the gathering and twisting of the filaments are performed upon a tightly wound package of thread. The package is preferably formed on a hollow perforated tube or spindle, the fiber being wound thereon directly from the so-called "cake" formed in the centrifuge pot of the spinning machine. During this winding operation no endeavor is made to wash the fiber or to treat it chemically, the purpose being to wind the thread in a closely compacted mass which is permeated by the solutions present in the spinning bath. At this time also, it is desirable to prevent drying of the thread. When the process is properly carried out, the amount of fiber present in the package forms only a small percentage of the total weight, the re-

mainder being made up of water and the salts of the precipitating bath. The subsequent operations of washing, desulphurizing, bleaching, sizing and dyeing etc. are carried out by forcing the various liquids under pressure through the package.

The structure of the package, due to the fact that the fiber forms only a small percentage of the total weight, allows the treating fluids readily to pass through the package while sufficient resistance is offered to the flow of the liquids, to insure a uniform penetration of the fluids to all parts of the thread mass. These operations are best carried out under pressure, in order that thorough contact at all parts of the thread may be effected, the compact winding of the thread preventing undue stresses on any parts thereof which might tend to weaken or destroy the fibers. After treatment, the package is dried in any suitable manner, but preferably by subjecting the package externally to the heat of an ordinary drying chamber while forcing hot air through the package from the interior outwardly so as to quickly dry the package uniformly by subjecting all parts of the package simultaneously to a uniform heat.

The rayon produced by the method of the present invention is characterized by its uniform properties, namely, its uniformity of color and luster as well as by its high strength.

The compacted package of twisted thread containing an interstitial filling of salt solution, forms in itself an important feature of the invention. The package is ready to be subjected to all subsequent operations for treatment of the fiber without necessity for skeining or for any of the special handling required under existing methods. The package, if kept in a moist condition, will retain its properties indefinitely, and will be ready for the subsequent operations of bleaching, washing, sizing, dyeing, etc. whenever it is necessary to prepare the thread for weaving or knitting purposes.

In the accompanying drawings Fig. 1 is a view in side elevation of a "cake" after being removed from the centrifuge pot. Fig. 2 is a view in side elevation of the package as it comes from the winding machine, a portion of the thread mass being broken away to show the perforated tube upon which the thread mass is supported. Fig. 3 is a detail view of a portion of an apparatus in which the packages may be subjected to the various solutions employed for treating the thread, illustrating the manner in which the packages may be supported to enable the solutions to be forced through the packages. Fig. 4 is a view in side elevation of the apparatus, a portion of which is illustrated in Fig. 3. Fig. 5 is a view in end elevation of a carriage forming a portion of a drying apparatus

which may be used in drying the packages, and Fig. 6 is a view in side elevation of the carriage illustrated in Fig. 5 and indicating also in cross section the walls of an ordinary drying chamber into which the carriage has been rolled.

The preferred form of the invention, which will now be described in detail, consists in the manufacture of rayon from viscose. The viscose or cellulose solution is produced from wood pulp or cotton linters or a combination of both in the usual manner. The fluid viscose is forced through a spinneret of any usual or preferred form into the precipitating bath which comprises a solution of sodium sulphate and dilute sulphuric acid. The filaments, after traversing a sufficient distance in the precipitating bath to cause complete formation of the fiber, are gathered together to form a thread or yarn. The yarn is passed out of the bath into a centrifuge pot of the usual form which rotates at a speed of several thousand revolutions per minute, the yarn being thrown out by centrifugal force and coiled in a cake within the pot. A cake formed in this manner is indicated at 7 in Fig. 1. The rotation of the centrifuge pot produces the necessary twist for retaining the filaments in thread formation. As thus far described, the process is similar to that usually carried out for the manufacture of rayon by the viscose method.

After the formation of the cake, it is removed from the pot and the thread is wound from the cake onto a suitable support to form a package. The support preferably consists of a hollow perforated tube, such as is indicated at 8 in Fig. 2 in order to permit the forcing of water or any other solutions through the package for purposes of washing, bleaching, sizing, dyeing, etc. The package is wound on a winding machine and during the universal winding operation, the yarn is maintained under a light tension but sufficient tension to form a compacted mass on the tube as indicated at 9 in Fig. 2. The solutions of the spinning bath which remain on the thread both in the cake and during the winding of the package are retained thereon so that when the package is completed, the entire mass of yarn is permeated by the solution. The cake, as formed in the centrifuge pot, is retained in a moist condition, and the winding of the package takes place with sufficient rapidity to prevent any appreciable evaporation of moisture. It is also desirable to maintain the package in moist condition as this prevents crystallization of the salts which would have a possible injurious effect on the fiber and furthermore, maintains the fiber as hydrocellulose rather than permitting it to be converted to oxycellulose which has been found less capable of taking the dye uniformly. When completed, the package comprises only a small proportion of its weight as fiber, usual-

ly 25% or less, the remainder being made up of water and the precipitating salts.

The package is now ready to be treated by the usual solutions employed for washing, desulphurizing, bleaching, oiling, sizing, dyeing, etc. The package may be kept as formed until any of these subsequent operations are to be performed. The washing is carried out by forcing water or suitable washing solution under pressure through the package. For uniform effect on all parts of the fiber, the washing is carried out alternately in opposite directions, from the interior of the tube outwardly and from the exterior of the tube inwardly. At the conclusion of the washing operation, the appearance of the package is not greatly different from its appearance when first wound from the centrifuge pot except that it is not quite so hard, although still tightly compacted.

An apparatus by which the washing can be carried out as above described is illustrated in Figs. 3 and 4. This apparatus comprises a tank 10 provided with a false bottom 11 and with a tightly fitting hinged cover 12 which may be securely bolted in closed position. The false bottom 11 divides the tank 10 into two chambers which communicate respectively with the pipes 13 and 14. Hollow perforated spindles 15 extend upwardly from the false bottom 11 and are adapted to support the perforated tubes 8 of the thread package as indicated in Fig. 3. The spindles 15 are closed at their upper ends and at their lower ends communicate with the chamber below the false bottom so that the washing solution can pass from one chamber of the tank to the other only through the perforated spindles. The packages are supported on the spindles by conical rubber washers indicated at 16 and these washers are arranged to prevent any flow of the washing solution between the upper chamber of the tank and the interior of the perforated spindles except through the thread mass. The washing solution is supplied from a tank indicated at 17. This tank communicates through a pipe 18 with a motor driven pump 19 and this pump is connected through a pipe 20 to a four-way valve 21. The pipes 13 and 14 lead to this valve as does also a pipe 22 through which the washing fluid is returned to the tank 17. The pump 19 supplies the washing solution to the valve 21 at the desired pressure and by means of the valve 21 the washing solution can be caused to flow alternately in opposite directions through the pipes 13 and 14 through the packages supported on the perforated spindles in the tank 10.

After washing, the package is subjected to the usual solutions for desulphurizing, bleaching, oiling, sizing, dyeing, etc. the yarn. These solutions may be such as are ordinarily employed in the viscose process

and may be applied in the same manner as the washing solution, that is by forcing them under pressure first in one direction and then in the other through the package, by means of the apparatus illustrated in Figs. 3 and 4. 70

The result of the above operations may be the production of bleached white rayon, which after drying, is satisfactory for commercial use. Where colored rayon is desired, a dyeing operation is performed on the 75 package either in addition to or in substitution for the bleaching treatment. In such case the dye is forced through the package alternately from the inside outwardly and from the outside inwardly under pressure 80 as in the washing operation. Although a slight amount of the precipitating salts, as well as some of the chemicals used for desulphurizing, may be present in the package during the dyeing operation, they are not 85 detrimental at this time, but in fact have a beneficial effect because they act somewhat in the nature of mordants to assist in the absorption of dye by the fiber. The dyeing step is carried out prior to any drying of the 90 yarn because, as previously stated, of the fact that crystallization of a large amount of the salts carried over from the precipitating bath, is likely to detract slightly from the high quality of the product. Drying of 95 the fiber prior to dyeing, has moreover the disadvantage that it permits conversion of the hydrocellulose of the yarn into oxycellulose which will not return to the hydrocellulose state if it again becomes wet. The hydrocellulose has been found to have a greater and more uniform affinity for the dye than oxycellulose and for this reason, it is desirable to prevent conversion of the yarn into its oxycellulose condition until after the 100 dyeing operation. By using a suitable sizing solution the thread while in the package may be prepared for use as warp thread in a loom without subjecting it to a separate sizing operation as is now the practice. The 105 thread can thus be wound directly from the package on to the beam of the loom, if desired, and the use of a separate sizing and winding mechanism eliminated. 110

The final operation consists in drying the 115 package. In this drying, it is desirable to subject all parts of the package simultaneously to heat in order that the package may be dried quickly and uniformly throughout and while under a uniform tension. As has been hereinbefore suggested, this drying is 120 preferably accomplished by forcing hot air through the package from the interior outwardly while subjecting the package externally to the heat of an ordinary drying chamber. An apparatus by which the packages can be conveniently dried in this manner is illustrated in Figs. 5 and 6. This apparatus comprises a carriage having a series of horizontally arranged hollow box- 125 130

like supports 23. Upon these supports are mounted any desired number of perforated spindles 24, a few only being shown in the drawing, similar to the spindles 15 of the apparatus illustrated in Figs. 3 and 4. These spindles are adapted to support the packages which are to be dried in the same manner that the packages are supported on the spindles 15. A pipe 25 connects with the interior of the supports 23 and this pipe is connected by a flexible hose 26 to a source of heated air. The heated air is forced into the supports 23 under pressure and passes into the spindles 24 and then outwardly through the packages. To subject the exterior of the packages to heat simultaneously with the application of the heat internally the carriage is run into the drying chamber of an ordinary drier indicated at 27 in Fig. 6 and for this purpose is conveniently mounted upon the wheels indicated at 28.

After drying, the package contains a loose winding of completed dyed, bleached or sized thread ready for use. Although the thread in the package is in a loosely wound condition, it is none the less regular and offers no difficulties in unwinding. The yarn may be wound from the package directly onto quills, bobbins, spools, or beams, suitable for use in weaving the thread into cloth.

It will be seen that the process of the present invention eliminates the repeated handling and harsh treatment necessary in prior methods and also permits treatment by the various washing and chemical solutions in such a manner that all parts of the thread or yarn are completely and uniformly effected.

The package of precipitated rayon wound from the centrifuge pot and containing only a small proportion of fiber, forms an important feature of the invention. If the yarn is not to be treated immediately or if it is desired to ship it to another place for treatment, the package may be easily transported or kept indefinitely until such time as the further operations are to be performed. It is desirable to keep the package in moist condition at all times until the final drying operation in order to prevent crystallization of any large quantity of the contained salts and also to maintain the fiber in its hydrocellulose condition.

The nature and objects of the invention having been indicated and the preferred manner of carrying out the invention having been specifically described what is claimed is:

1. The process of manufacturing rayon which consists in forming in a precipitating bath a plurality of filaments from a cellulose solution, gathering the filaments into a thread, winding up the thread as it comes from the precipitating bath, rewinding the wet thread under tension onto a perforated tube to form a compacted package consist-

ing of a small proportion of fiber and a relatively large proportion of water and substances from the precipitating bath, washing the package and subjecting the package to the action of a solution for determining the color of the thread by forcing solutions through the package under pressure, and drying the package.

2. The process of manufacturing rayon which consists in forming in a precipitating bath a plurality of filaments from a cellulose solution, gathering the filaments into a thread, winding up the thread as it comes from the precipitating bath, rewinding the wet thread under tension onto a perforated tube to form a compacted package consisting of a small proportion of fiber and a relatively large proportion of water and substances from the precipitating bath, washing the package and subjecting the package to the action of a dyeing solution by forcing solutions through the package under pressure and drying the package.

3. The process of manufacturing rayon which consists in forming in a precipitating bath a plurality of filaments from a cellulose solution, gathering the filaments into a thread, winding up the thread as it comes from the precipitating bath, rewinding the wet thread under tension onto a perforated tube to form a compacted package consisting of a small proportion of fiber and a relatively large proportion of water and substances from the precipitating bath, washing the package and subjecting the package to the action of solutions to prepare the thread for use by forcing solutions through the package under pressure and drying the package.

4. The process of manufacturing rayon which consists in forming in a precipitating bath a plurality of filaments from a cellulose solution, gathering the filaments into a thread, winding up the thread as it comes from the precipitating bath, rewinding the wet thread under tension onto a perforated tube to form a compacted package consisting of a small proportion of fiber and a relatively large proportion of water and substances from the precipitating bath, washing the package and subjecting the package to the action of a bleaching solution by forcing solutions through the package under pressure and drying the package.

5. The process of manufacturing rayon which consists in forming in a precipitating bath a plurality of filaments from a cellulose solution, gathering the filaments into a thread, winding up the thread as it comes from the precipitating bath, rewinding the wet thread under tension onto a perforated tube to form a compacted package consisting of a small proportion of fiber and a relatively large proportion of water and substances from the precipitating bath, washing the package and subjecting the package to the

action of a sizing solution by forcing solutions through the package under pressure, and drying the package.

6. The process of manufacturing rayon which consists in forming in a precipitating bath a plurality of filaments from a cellulose solution, gathering the filaments into a thread, twisting and winding the thread into a cake, winding the wet thread under tension from the cake onto a perforated tube to form a compacted package consisting of a small proportion of fiber and a relatively large proportion of water and substances from the precipitating bath, washing the package by forcing water through the package under pressure and drying the package.

7. The process of manufacturing rayon which consists in making a viscose solution, forming filaments from the viscose by precipitating it in a salt bath, gathering the filaments into a thread, twisting and winding the thread into a cake, winding the wet thread under tension from the cake onto a perforated tube to form a package consisting of a small proportion of fiber and a relatively large proportion of water and dissolved salts, washing the package by forcing water under pressure therethrough, and drying the package.

8. The process of manufacturing rayon from viscose which consists in precipitating viscose in a salt bath to form a plurality of filaments, gathering the filaments into a thread, twisting and winding the thread into a cake, winding the thread while wet and containing salts from the precipitating bath from the cake onto a perforated tube to form a package, washing and dyeing the package by forcing solutions through the package under pressure, and finally drying the package.

9. The process of manufacturing rayon from viscose which consists in winding the precipitated thread without drying or other treatment into a compacted package, washing and dyeing the package, maintaining the package in a moist condition until after the dyeing operation and finally drying the package.

10. The process of preparing rayon which consists in forming a plurality of filaments from viscose in a sulphuric acid and sodium sulphate precipitating bath, gathering the filaments into a thread, twisting the thread and winding it onto a hollow cylinder or "cake", winding the thread while moist from the cake onto a hollow perforated tube to form a compact package consisting of a small proportion of fiber and a relatively large pro-

portion of water and substances from the precipitating bath, washing and dyeing the package by forcing solutions through the package under pressure and finally drying the package.

11. The process of preparing rayon which consists in forming a plurality of filaments from viscose in a sulphuric acid and sodium sulphate precipitating bath, gathering the filaments into a thread, twisting the thread and winding it into a hollow cylinder or "cake", winding the thread while moist from the cake onto a hollow perforated tube to form a compact package consisting of a small proportion of fiber and a relatively large proportion of water and substances from the precipitating bath, washing the package by forcing washing liquids through the package alternately from within outwardly and from without inwardly, dyeing the package by forcing a dyeing solution through the package, maintaining the package in a moist condition until after the dyeing operation, and finally drying the package.

12. The process of preparing rayon which consists in forming a plurality of filaments from viscose in a sulphuric acid and sodium sulphate precipitating bath, gathering the filaments into a thread, twisting the thread and winding it into a hollow cylinder or "cake", winding the thread while moist from the cake onto a hollow perforated tube to form a compact package consisting of a small proportion of fiber and a relatively large proportion of water and substances from the precipitating bath, washing the package, subjecting the package to the action of solutions to prepare the thread for use and finally drying the package.

13. The process of manufacturing rayon which consists in forming a plurality of filaments from viscose in a sulphuric acid and sodium sulphate precipitating bath, gathering the filaments into a thread, winding the precipitated thread while wet and containing salts from the precipitating bath onto a perforated tube to form a package, consisting of a small proportion of fibre and a relatively large proportion of water and dissolved salts, washing and dyeing the package by forcing solutions through the package under pressure, maintaining the package in a moist condition until after the dyeing operation, and finally drying the package.

In testimony whereof I have signed my name to this specification.

ISAAC B. MERRIMAN.